

# UNITED STATES PATENT OFFICE.

LOUIS S. ROSS, OF NEWTONVILLE, MASSACHUSETTS.

## TIME-BURNING RAILWAY SIGNAL-FUSEE.

1,359,922.

Specification of Letters Patent. Patented Nov. 23, 1920.

No Drawing. Original application filed August 29, 1916, Serial No. 117,551. Divided and this application filed September 20, 1917. Serial No. 192,335.

To all whom it may concern:

Be it known that I, Louis S. Ross, a citizen of the United States, and a resident of Newtonville, in the county of Middlesex and 5 State of Massachusetts, have invented an Improvement in Time-Burning Railway Signal-Fusees, of which the following description is a specification.

This application is a division of my co-pending application Serial No. 117,551, filed 10 August 29, 1916.

This invention relates to time burning, railway signal fusees. An important purpose of my invention is to construct a time burning railway signal fusee in such manner that it can be kept for a long while without deteriorating or absorbing moisture, and will retain unimpaired its quality of ready ignition, brilliancy, tenacity and force of flame.

15 Railway fusees which are designed as signals to be thrown from the end of a moving train or to be placed on the track at the rear of the train or otherwise are made of a mixture of chemicals, including usually a chlorate or perchlorate, sulfur, carbonaceous material, and some oxidizing metallic nitrate, which burns with a colored flame. The ingredients are mixed and packed in a stout fiber or paper tube. In order that my invention may be readily understood, I give 20 here a typical formula of a fusee, which formula is taken from my Patent No. 1,059,214, dated April 15, 1913. It will be understood, however, that my invention is not in any way limited to the exact character or proportions of ingredients set forth in this formula, and that I simply quote it here by way of example and in order to facilitate 25 comprehension of my invention.

30 Metallic nitrate----- 72 parts.  
Sulfur----- 12 "  
Hydrocarbon----- 6 "  
Potassium perchlorate--- 12 "

35 Fusees at the present time are made in most substantial quantities without the use of a chlorate, a perchlorate being substituted in general practice.

The railroads of the United States and 40 the Interstate Commerce Commission co-operate together in maintaining a bureau known as the Bureau for the Safe Transportation of Explosives and other Dangerous Articles, and fusees are subject to the 45 specifications of this bureau. Fusees, such

as described and heretofore manufactured fulfil these requirements in so far as they relate to easy ignition, brilliancy and force of flame under adverse conditions, but they are subject to deteriorating influences when 60 kept due to the chemicals absorbing moisture. This is particularly noticeable during the summer months with high humidity conditions.

One cause of deterioration is that the metallic nitrate which constitutes a large proportion of the charge of the fusee is very deliquescent, particularly nitrate of strontium which is used in making red fusees, while nitrate of barium is used in making 65 green fusees, or sodium salts in making yellow fusees, and when the fusee stands will absorb water from the air and impair the quality of the pyrotechnic mixture. It has been attempted to protect the charge from 70 moisture by paraffining the outer paper casting of the fusee but this operation lacks the necessary efficiency and is expensive to carry out.

Another cause of deterioration in these 75 mixtures is the fact that when chlorate is used instead of perchlorate or even when mixed with perchlorate, that the chlorate and sulfur will re-act upon each other when subjected to dampness and spontaneous 80 ignition results.

The danger of chlorate mixtures with sulfur has been long recognized by railroads, due to the danger of spontaneous ignition 85 and the Bureau of Explosives in its specifications limits their use by the following rule: "Fusees containing sulfur must not contain more than 2.6% of potassium chlorate or an equivalent amount of any other chlorate. Fusees containing chlorates in any 90 quantity must not contain any ammonium salts."

The danger has long been known and was 95 overcome in some degree by the addition of an anti-acid or neutralizing agent to the chlorate sulfur mixtures, as described in Patent No. 1,019,190 dated March 5, 1912. The present bureau specifications on fusees 100 require the use of a perchlorate which is somewhat less efficient and more expensive 105 than the chlorate.

My invention proposes to overcome the 110 danger of spontaneous ignition whether the fusee is made in whole or only in part with chlorate. The danger of spontaneous com-

bustion may indeed be minimized or substantially eliminated by the use of perchlorate to the exclusion of chlorate but the results obtained are disastrous as far as efficiency 5 and reliability go and if the fusee has been subjected to the natural moisture of humidity of the air, particularly in moist climates, the fusee which burns the required time with brilliancy and force of flame when first made 10 will absolutely fail to give an easily distinguishable signal when subjected to moist storage conditions for even a few weeks and in many cases the moisture absorbed is so great as to cause the fusee to extinguish itself 15 due to excessive moisture.

In accordance with my invention, I protect the particles of deliquescent material, such for example, as nitrate of strontium from contact with the air by providing each 20 with a coating which will resist the access of moisture thereto but will not impair the burning qualities of the fusee. For this purpose a suitable fat or wax such as petroleum grease or paraffin may be utilized. This is 25 preferably applied to the materials in the following manner:

The nitrate of strontium or of barium or other deliquescent ingredient used is first warmed in a drying pan, steam-jacketed 30 kettle or other device in which it may be thoroughly warmed, and then is mixed mechanically with a small quantity of suitable water-proofing material such as described and which will not interfere with the burning 35 of the finished product, and until each particle of the nitrate is separately coated with said waterproofing material. In fact the addition of suitable waxy or fatty matter will even improve the burning quality. 40 It will be apparent that by this mixing the various particles of the metallic salt will be covered with a slight coating which will effectually prevent moisture from the air being taken up thereby.

45 It has been customary in the manufacture of these devices to add as an ingredient some carbonaceous material, such for example as sawdust treated with grease, the quantity being determined by experiment. Evidently 50 less grease may be used in mixing the sawdust and a corresponding amount utilized in waterproofing the deliquescent salt. The keeping qualities of the fusee will thus be greatly improved without necessarily altering 55 the proportions found by experience to be most advantageous. I have found, however, that the same mixtures can be used together with an additional amount of waterproofing material applied to the deliquescent 60 salts.

I have previously referred to the danger of sulfur and chlorate when in contact with moisture and in order to prevent interaction of the sulfur and chlorate used which 65 might lead to spontaneous ignition, it is

possible to treat the sulfur or the chlorate or both in a similar manner and I preferably do so. In this case a light coating of inert inflammable material covers the various particles and effectually insulates one ingredient from the other and prevents a chemical reaction from beginning before the fusee is purposely ignited. A coating of waxy or fatty material on the particles of sulfur will also prevent oxidization thereof 70 to initiate acid reactions and I preferably so coat the said sulfur particles. I am thus able to use either chlorate or perchlorate alone or both together in any suitable proportions. In other words, I utilize salt of 80 suitable oxygen and chlorin bearing acids.

Where in the claims I refer to a chlorate, I include perchlorates and other chlorates.

The coated particles of the nitrate are only coated in a loose condition, permitting 85 the mixing thereof with the other ingredients of the fusee, such as sulfur and chlorate.

Since I have described in so much detail one embodiment of my invention, I should point out that the exact nature and quantity 90 of the ingredients and the exact manner of their treatments as described herein are not essential but merely typical and that what I do claim and desire to secure by Letters Patent is:

1. A time burning, railway signal fusee comprising in combination; metallic nitrate, all the particles whereof are separately slightly coated with a waterproofing, inflammable material, thereby preventing the absorption of moisture by said metallic nitrate; sulfur; and a small quantity of chlorate mixed and packed in a suitable tube, said fusee being thereby rendered capable of being kept for a prolonged period 100 without absorbing moisture, deteriorating or impairing the burning qualities of said ingredients. 105

2. A time burning, railway signal fusee comprising in combination; metallic nitrate, 110 all the particles whereof are separately slightly coated with a waterproofing, inflammable material, thereby preventing the absorption of moisture by said metallic nitrate; sulfur; and a small quantity of a 115 chlorate not exceeding 2.6% of the mixture, said materials being mixed and packed in a suitable tube, said fusee being thereby rendered capable of being kept for a prolonged period without absorbing moisture, deteriorating or impairing the burning qualities 120 of said ingredients.

3. A time burning, railway signal fusee comprising in combination; metallic nitrate, all the particles whereof are separately 125 slightly coated with a small quantity of hydrocarbon, thereby preventing the absorption of moisture by said metallic nitrate; sulfur; and a small quantity of a chlorate, said ingredients being mixed and packed 130

in a suitable tube, said fusee being thereby rendered capable of being kept for a prolonged period without absorbing moisture, deteriorating or impairing the burning qualities of said ingredients.

4. A time burning, railway signal fusee comprising in combination; metallic nitrate, all the particles whereof are separately slightly coated with a small quantity of 10 paraffin, thereby preventing the absorption of moisture by said metallic nitrate; sulfur; and a small quantity of a chlorate, said ingredients being mixed and packed in a suitable tube, said fusee being thereby rendered 15 capable of being kept for a prolonged period without absorbing moisture, deteriorating or impairing the burning qualities of said ingredients.

5. A time burning railway signal fusee 20 comprising in combination; metallic nitrate, all the particles whereof are separately slightly coated with a small quantity of hydrocarbon, thereby preventing the absorption of moisture by said metallic nitrate; sulfur; 25 and a small quantity of a chlorate, the par-

ticles of said chlorate being also separately slightly coated with hydrocarbon, said ingredients being mixed and packed in a suitable tube, said fusee being thereby rendered capable of being kept for a prolonged 30 period without absorbing moisture, deteriorating or impairing the burning qualities of said ingredients.

6. A time burning railway signal fusee comprising in combination; metallic nitrate, 35 all the particles whereof are separately slightly coated with a waterproofing, inflammable material, thereby preventing the absorption of moisture by said metallic nitrate; sulfur; and a small quantity of 40 chlorate, said ingredients being mixed and packed in a suitable tube, said fusee being thereby rendered capable of being kept for a prolonged period without absorbing moisture, deteriorating or impairing the 45 burning qualities of said ingredients.

In testimony whereof I have signed my name to this specification.

LOUIS S. ROSS.